

# UNITED STATES PATENT OFFICE.

JAMES HENRY RICKER, OF FORT WORTH, TEXAS, ASSIGNOR OF TWO-THIRDS TO SAMUEL PERCIVAL GREENE AND JOHN ALFRED TORNEY EVANS, OF FORT WORTH, TEXAS.

## FUEL COMPOUND.

SPECIFICATION forming part of Letters Patent No. 707,722, dated August 26, 1902.

Application filed February 8, 1902. Serial No. 93,197. (No specimens.)

*To all whom it may concern:*

Be it known that I, JAMES HENRY RICKER, a citizen of the United States, residing at Fort Worth, in the county of Tarrant and State of Texas, have invented a new and useful Fuel Compound Known as "Ricker's Crude-Oil Brick Fuel," of which the following is a specification.

This invention relates to fuel, and has for its object to provide an improved composition of matter producing a fuel as a substitute for coal and to have the fuel in such form as to be conveniently handled in transportation and in using the same in grates, stoves, and furnaces, and in any way that coal can be used, furnishing a fuel absolutely non-explosive, equal, if not superior, to the best grade of bituminous coal at a less cost.

The fuel consists of the following thoroughly-mixed ingredients, by volume: crude petroleum, eighteen and three-fourths per cent.; rosin, two and one-half per cent.; sawdust, twelve and one-half per cent.; clay, twelve and one-half per cent.; liquid glass, two and one-half per cent.; lignite or coal-dust, fifty-one and one-fourth per cent.; total, one hundred per cent., the resilient compound being put up loosely in bulk and also pressed into bricks or cakes or any other form desired. It will also be observed that the oil, rosin, sawdust, and lignite or coal-dust form highly-combustible component parts of the fuel, the liquid glass and clay serving as a bond between the other ele-

ments. The clay also forms in part a body 35 for the fuel to hold and maintain the heat when the other parts begin to decrease in temperature and also to prevent too rapid burning of the combustible parts of the compound, the rosin uniting with the other parts 40 to sustain the combustion.

The present fuel is in such form as to be conveniently handled and, furthermore, is non-explosive. It will furthermore be understood that the rosin, sawdust, and lignite 45 or coal-dust are in powdered form, the three last-named elements forming a vehicle for the crude petroleum-oil and the liquid glass and the clay binding the compound together, the clay forming in part a body for the same. 50

What is claimed is this:

An artificial fuel consisting of the following thoroughly-associated ingredients, by volume, in about the proportions as follows: Crude petroleum eighteen and three-fourths 55 per cent., rosin two and one-half per cent., sawdust twelve and one-half per cent., clay twelve and one-half per cent., liquid glass two and one-half per cent. and lignite or coal-dust fifty-one and one-fourth per cent. 60

In testimony that I claim the foregoing as my own I have hereto affixed my signature in the presence of two witnesses.

JAMES HENRY RICKER.

Witnesses:

Wm. J. BISHOP,  
SALLYE SIMPSON.